

# UNITED STATES PATENT OFFICE.

WILLIAM L. RICE, OF READING, PENNSYLVANIA, ASSIGNOR OF ONE-HALF TO HIMSELF  
AND ONE-HALF TO PETER S. BRAUCHER, OF READING, PENNSYLVANIA.

## SOFT-METAL ALLOY AND METHOD OF MAKING SAME.

1,269,000.

Specification of Letters Patent. Patented June 11, 1918.

No Drawing.

Application filed June 27, 1916. Serial No. 106,084.

To all whom it may concern:

Be it known that I, WILLIAM L. RICE, a citizen of the United States of America, and resident of Reading, in the county of 5 Berks and State of Pennsylvania, have invented a certain new and useful Improvement in Soft-Metal Alloys and Methods of Making Same, of which the following is a true and exact description.

10 The object of my present invention is to provide an improved alloy suitable for use as a soft metal bearing metal.

The distinguishing characteristic of my invention is the presence in the improved 15 alloy of a sodium content secured by adding caustic soda to the other constituents of the alloy before melting, or while in a molten condition. The addition of the caustic soda to the ordinary constituents of a 20 soft bearing metal appears to harden and toughen the resultant product, to insure better lubrication with ordinary lubricants, and to reduce the liability of the bearings to fail from overheating.

25 An important practical advantage of the invention when used in connection with the common type of soft bearing metal comprising as its principal constituents, lead, tin and antimony, is that its use permits

30 of the formation of a satisfactory bearing metal containing less of the relatively expensive hardening and toughening tin and antimony constituents, and more of the less expensive lead constituent than would 35 otherwise be required. The addition of the sodium content to the bearing metal not only hardens and toughens the latter, but makes it somewhat hygroscopic in character, and this in itself seems to improve the 40 character of the lubrication obtained with oil or other ordinary lubricants.

The amount of the sodium content, and the character of the other bearing metal constituents employed may vary widely, 45 but without loss of the characteristic advantages had from the use of the caustic soda. One example of an alloy formed in accordance with the present invention and which has given excellent results in practice when used in bearings for railway car

50 journals, is an alloy formed from lead, tin,

antimony and caustic soda in the following proportions:

|              |           |    |
|--------------|-----------|----|
| Lead         | 88 parts. | 55 |
| Tin          | 6 "       |    |
| Antimony     | 3½ "      |    |
| Caustic soda | 2½ "      |    |

The constituents mentioned may be mixed together before melting, but advantageously I form a molten mixture of tin and antimony and add thereto a portion of the caustic soda to be used, and then add the product thus obtained to molten lead, and add to the last mentioned mixture the remainder of the caustic soda to be used. Advantageously a small amount of copper sulfate, say from one-quarter to one part may be added to act as a flux in effecting an efficient mixture. 70

It is my belief that in the resultant product, the sodium is present as metallic sodium held in a solidified solution of lead, antimony and tin, but whether or not I am right in this there is no question as to the 75 practical improvement in soft bearing metals had by the use of the present invention.

It is to be understood that my invention in its broader aspects is not limited to soft 80 bearing metal alloys of the particular composition or constituents hereinbefore mentioned. For example, it may well be used with a bearing metal alloy containing zinc as well as tin and antimony in addition to 85 the lead constituent.

Having now described my invention, what I claim as new and desire to secure by Letters Patent, is:

1. An alloy consisting of lead, tin, antimony and sodium. 90

2. An alloy formed by solidifying a molten mixture of lead, tin, antimony and caustic soda.

3. The method of forming a soft metal 95 alloy which consists in adding caustic soda to a molten mixture of tin and antimony, and then effecting a molten mixture of the product with lead and adding caustic soda thereto.

WILLIAM L. RICE.

Copies of this patent may be obtained for five cents each, by addressing the "Commissioner of Patents, Washington, D. C."